

3,352,694

LOW TEMPERATURE METALLIZING PAINT  
AND METHOD OF MAKING SAME

Leonard Reed, San Jose, and Donald C. Figone, San Francisco, Calif., assignors, by mesne assignments, to Varian Associates, a corporation of California  
No Drawing. Filed June 17, 1963, Ser. No. 288,454  
10 Claims. (Cl. 106—1)

This invention relates to a metallizing paint composition. More particularly, this invention relates to a low temperature metallizing paint composition for obtaining a vacuum tight metallized surface on ceramic bodies and the method of obtaining the metallizing paint.

Generally, a ceramic body is metallized by painting the portion of the ceramic body to be metallized with a metallizing paint and then heating the coated ceramic to sinter a refractory metal, present in the paint, onto the ceramic. The resulting metallized layer generally comprises a refractory metal phase which is extensively penetrated by a non-metallic "glassy" phase that wets and adheres to both the refractory metal and the ceramic body. The metallizing paint may comprise a vehicle which includes a binder and a solvent with the refractory metal and the "glassy" phase material suspended therein. The metallizing paint is applied to the ceramic body by hand painting, spraying, dipping, silk screening or by any other suitable means. Heretofore in the prior art, the high sintering temperature (1300 to 1600° C.) of many metallizing paints has tended to warp various ceramic bodies. Also, expensive apparatus, such as high temperature furnaces, etc. are required to produce these high sintering temperatures.

Therefore, an object of this invention is to provide a low temperature metallizing paint.

Another object of this invention is to provide a metallizing paint having a sintering temperature of about 1000° C.

Still another object of this invention is to provide a metallizing paint having a sintering temperature of about 1000° C. for producing a vacuum tight metallized layer on ceramic bodies.

A further object of this invention is to provide a method for obtaining a low temperature metallizing paint.

These and other objects of this invention are obtained by a metallizing paint composition which includes at least one material therein which acts to reduce the sintering temperature of the refractory metal and the melting temperature of the "glassy" phase material contained in the metallizing paint. In accordance with this invention, a low temperature metallizing paint composition comprises a vehicle including a binder in a solvent. A plurality of metal powders are dispersed in the vehicle and include a refractory metal and a quantity of at least one metal which reduces the sintering temperature of the refractory metal and the melting temperature of "glassy" phase material. A plurality of "glassy" phase producing powders are also dispersed in the vehicle. Also, a non-metallic powder, such as boric acid, may be added to the vehicle to further aid in reducing the melting temperature of the "glassy" phase material. Further, the powders in the vehicle may be at least partially coated with iron to improve the density of the sintered refractory metal layer obtained with the metallizing paint.

This invention, as well as other objects, features and advantages thereof, will be readily apparent from the following detailed description. In accordance with this invention, a low temperature metallizing paint is obtained by preparing a vehicle which includes a solvent and a binder. A preferred binder material is nitrocellulose. However, the binder material may be any organic film-

forming substance, such as ethyl cellulose or methacrylate resin, commonly used and well known in the art, which decompose upon heating leaving little or no residue. A plurality of metal powders are placed in the vehicle and include a refractory metal selected from the group consisting of tungsten, molybdenum and rhenium and a quantity of at least one metal, selected from the group consisting of copper, nickel, cobalt and iron, for reducing the sintering temperature of the refractory metal and the melting temperature of "glassy" phase producing material. For purposes of describing and claiming the present invention, "metal powders" are defined as any one or more of the various powder forms of metal, such as pure metal powder, metal oxide powder, metal hydride powder, etc. A plurality of non-metallic "glassy" phase producing powders are also placed in the vehicle and include by weight a majority of manganese dioxide and a minority by weight of silica, and titanium dioxide. Also, a non-metallic powder, preferably boric acid, may be added to the vehicle to further aid in reducing the melting temperature of the "glassy" phase material. A uniform distribution or suspension of the powders in the vehicle is obtained by ball milling the metallizing paint mix.

According to a preferred example of the present invention, a low temperature metallizing paint composition having a sintering temperature of about 1000° C. is formed by preparing a vehicle which includes a binder and a solvent. One hundred cc. by weight of a preferred solvent comprises about 50 cc. of ethylene glycol monoethyl ether, such as Dowenol EE, and 50 cc. of methyl-ethyl ketone. The vehicle is formed by adding by weight about 1.5 grams of nitrocellulose to 100 cc. of the solvent. A plurality of at least —325 mesh metal oxide powders are added to the 100 cc. of vehicle and include by weight about 100 to 150 grams of a refractory metal selected from the group consisting of tungsten oxide, molybdenum oxide or rhenium oxide and about 10 grams nickel oxide, about 5 grams of copper oxide and about 2 grams of iron oxide. The nickel, copper and iron oxides act to reduce the sintering temperature of the refractory metal, which is preferably tungsten oxide, and also reduce the melting temperature of the "glassy" phase materials described hereinbelow. A plurality of at least —325 mesh "glassy" phase producing powders are also added to the 100 cc. of vehicle and include about 10.4 grams of manganese dioxide, about 4.4 grams of silica, and about 2.2 grams of titanium dioxide. Also, about 4.2 grams of boric acid is added to the vehicle to aid in reducing the melting temperature of the "glassy" phase material.

A uniform distribution or dispersion of the powders in the vehicle is obtained by ball milling the metallizing paint mix for approximately 48 hours. In order to increase the hardness and density of the metallized layer produced by the metallizing paint, the ball milling is performed in an iron ball mill with 1/2 inch diameter iron balls which intimately coats at least a portion of the powder particles dispersed in the vehicle with iron from the iron balls by a disintegration commutation process.

The metallizing paint may be applied to any suitable ceramic, such as a beryllium oxide ceramic or a high alumina ceramic, that is, one containing at least 85% alumina. The sintering temperature of the metallizing paint is about 1000° C. The sintering preferably takes place for 1/2 hour in an atmosphere of four parts nitrogen to one part hydrogen having a dew point of plus 1000° F. This low sintering temperature is due to the materials used, such as the copper, nickel and iron. In the absence of these materials, the sintering temperature of the metallizing paint would be in the vicinity of 1500 to 1600° C. It is believed that the presence of the copper, nickel and

iron powders intermingled with the refractory metal powder causes this reduction in the sintering temperature of the refractory metal. Also, a portion of the copper, nickel and iron exist in ionic form in the "glassy" phase melt during sintering and reduce the melting temperature of the "glassy" phase material, that is, the manganese, silica and titanium oxides. The boric acid further aids in reducing the melting temperature of the "glassy" phase material. The metallizing paint composition described hereinabove in detail is such that at about 1000° C. the "glassy" phase materials produce a manganese-titanium-alumino-borosilicate melt that extensively penetrates the refractory metal and wets and adheres to both the refractory metal and the ceramic to form a vacuum tight metallized surface on the ceramic body. Tensile strengths up to 12,000 p.s.i. have been obtained by utilizing this metallizing paint in conjunction with an overplate of nickel followed by a copper-silver braze to a copper metal member.

Although specific quantities of the materials comprising a novel low temperature metallizing paint are given hereinabove, it is to be understood that these quantities may be varied according to the paint characteristics desired without departing from the spirit and scope of the present invention. For example, the metal oxide powders may be replaced by pure metal powders. Also, the boric acid need not be used in which case the metallizing paint will have a sintering temperature of about 1000 to 1100° C. Further, the consistency of the paint desired may be controlled by varying the amounts of the solvent and binder used. Also, cobalt oxide may be used in place of the nickel and/or copper oxide; and other "glassy" phase producing materials may be used rather than the manganese, silica and titanium described hereinabove.

What is claimed is:

1. A metallizing paint for producing a vacuum-tight metallized surface on ceramic, said metallizing paint having a sintering temperature of about 1000° C. comprising: a vehicle including a binder and a solvent; a plurality of metal powders dispersed in said vehicle, said metal powders consisting essentially of approximately 85% to 90% by weight of a refractory metal selected from the group consisting of tungsten, molybdenum and rhenium, and approximately 10% to 15% by weight of at least one other metal selected from the group consisting of nickel, copper, cobalt and iron; and a plurality of "glassy" phase producing powders dispersed in said vehicle.
2. Claim 1 wherein said refractory metal is in oxide form.
3. Claim 1 wherein said other metal is in oxide form.
4. Claim 1 wherein said other metal consists of approximately 60% nickel, approximately 30% copper and approximately 10% iron by weight.
5. Claim 1 wherein said "glassy" phase producing pow-

ders consist essentially of a majority by weight of manganese dioxide and a minority by weight of silica and titanium dioxide.

6. Claim 1 wherein said "glassy" phase producing powders consist essentially of approximately 60% of manganese dioxide, 26% silica and 14% titanium dioxide by weight.

7. Claim 1 further including boric acid to reduce the melting temperature of the "glassy" phase producing powders.

8. Claim 7 wherein the proportion of "glassy" phase producing powders to boric acid is approximately 4:1 by weight.

9. Claim 1 wherein the metal powders and the "glassy" phase producing powders are at least partially coated with iron.

10. The method of making a metallizing paint having a sintering temperature of about 1000° C. comprising the steps of:

- 20 preparing a vehicle by combining a binder with a solvent;
- 25 placing in the vehicle a plurality of metal powders consisting essentially of a refractory metal selected from the group consisting of tungsten, molybdenum and rhenium and a quantity of at least one metal selected from the group consisting of cobalt, nickel, copper and iron;
- 30 placing in the vehicle a plurality of "glassy" phase producing powders; and
- 35 coating the powder particles in the vehicle with iron such as by ball-milling the vehicle containing the powders with iron balls.

#### References Cited

#### UNITED STATES PATENTS

|           |         |                                  |
|-----------|---------|----------------------------------|
| 869,013   | 10/1907 | McOuat.                          |
| 1,947,112 | 2/1934  | Ruben.                           |
| 2,100,425 | 11/1937 | Bent et al. ----- 106—187        |
| 2,160,133 | 5/1939  | Ellis ----- 106—187 XR           |
| 2,461,878 | 2/1949  | Christensen et al.               |
| 2,488,731 | 11/1949 | Lambert et al.                   |
| 2,530,217 | 11/1950 | Bain.                            |
| 2,750,657 | 6/1956  | Herbert et al.                   |
| 2,759,446 | 8/1956  | Ewing.                           |
| 2,985,547 | 5/1961  | Luks ----- 117—160               |
| 3,093,490 | 6/1963  | MacKay ----- 106—1               |
| 3,110,571 | 11/1963 | Alexander ----- 117—160 X        |
| 3,189,504 | 6/1965  | Whittle et al. ----- 156—234     |
| 3,227,591 | 1/1966  | Lambert et al. ----- 156—80      |
| 3,290,171 | 12/1966 | Zollman et al. ----- 106—1       |
| 3,293,072 | 12/1966 | Doolittle et al. ----- 117—138,8 |

55 ALEXANDER H. BRODMERKEL, Primary Examiner.

J. H. WOO, Assistant Examiner.